

## UNITED STATES PATENT OFFICE.

CLETUS F. CHOSA, OF MILWAUKEE, WISCONSIN, ASSIGNOR TO THE CUTLER-HAMMER MFG. CO., OF MILWAUKEE, WISCONSIN, A CORPORATION OF WISCONSIN.

## COMPOSITION MATERIAL ADAPTED TO THE PLASTIC ART.

No Drawing.

Application filed June 18, 1923. Serial No. 646,235.

This invention relates to composition materials adapted to the plastic art; also to methods of producing such materials.

In prior Patent No. 1,233,416, issued July 5 17, 1917, to William H. Steinberg, is disclosed a composition material comprising an inert base or filler, a polymerizing or vulcanizing agent and a binder including coal tar pitch, stearine pitch, an animal or vegetable oil capable of polymerization and a solvent of low boiling point, together with methods of producing such material. Also in a prior application of Clarence A. Nash, filed July 19, 1920, Serial No. 397,181, are 10 15 disclosed certain improvements in the product and process of Steinberg.

The present invention has among its objects that of otherwise and further improving the product set forth in said Steinberg 20 patent.

Another object is that of providing improved and simplified methods of producing materials adapted to the uses contemplated in said Steinberg patent.

Another object is that of providing a 25 novel and improved material adapted to the plastic arts.

Another object is that of providing improved and simplified methods of producing such material.

Other objects and advantages will herein-after appear.

While the materials and processes disclosed in said patent and also the improved process and product disclosed in said application have proven of great value and have been extensively used industrially, the processes aforesaid have been unduly complicated, expensive and time consuming, where- 35 40 45 as by the new process herein contemplated it has been found possible not only to simplify the method of production of the material as well as reduce the time, labor and expense involved in production thereof but also to produce a superior product.

According to the teaching of the Steinberg patent, a relatively inert filler material such for example as asbestos, is impregnated with a composition binder comprising 50 55 among other ingredients approximately equal portions of stearine pitch and coal tar pitch, these substances constituting the major constituents of the binder. In the application of Nash, a portion of the coal tar pitch is replaced by an asphaltic body such

for example as gilsonite whereas certain further variations and improvements not herein important are contemplated.

However, both said patent and said application contemplate the use in the binder 60 of very substantial proportions of coal tar pitch and this substance, under the treatment imposed, precipitates large quantities of carbon which if permitted to remain in situ has been found quite deleterious to the 65 product in matters of strength and the like. Therefore both the patent and application aforesaid teach as an important step in their respective processes that of removing such free carbon which as stated is likely to 70 be precipitated to the extent of 30% by weight of the coal tar pitch employed, whereas in practice it is now known that this amount of free carbon may and frequently does approximate 50% by weight of the coal 75 tar pitch.

This procedure obviously involves loss of a relatively high percentage of the material since the carbon so removed is of little or no commercial value. Also the steps necessary 80 for such removal are quite difficult, expensive and time consuming, since the carbon has a tendency to settle and adhere to the lower portions of the tank, still or the like in which the binder is formed, necessitating 85 considerable labor for its removal, whereas the container is frequently very much damaged by the rough treatment incident to such removal.

According to the herein contemplated 90 method, I am able to obviate entirely the aforementioned procedure for removal of free carbon, whereas, as a result of the aforesaid method I am also able to obtain a product adapted to all or practically all uses to 95 which the earlier products are applicable and moreover possessing advantages there-over.

Thus in accordance with the herein contemplated procedure suitable proportions of 100 stearine pitch and asphaltic body may be brought together in the absence of coal tar pitch, or in the absence of a sufficient quantity of the latter to involve precipitation of a material quantity of carbon under the 105 treatment imposed, the resultant mixture being thereafter treated, under suitable conditions of temperature, with a quantity of a solidifiable substance such for example as castor oil, China wood oil or the like and a 110

quantity of an agent, such as sulphur, adapted to promote induration under the influence of heat, to produce a molding compound or a binder therefor. Additionally a 5 quantity of a suitable plasticizing agent such for example as iron oxide may be preferably included to promote flow and generally to facilitate molding of the material.

10 In those cases wherein a relatively inert filler, such for example as comminuted asbestos, is incorporated with the aforescribed plastic material prior to molding thereof the sulphur or other solidifying 15 agent may be preferably mixed with such filler prior to incorporation.

The aforescribed plastic material, preferably after incorporation with a suitable filler, is thereafter adapted to form giving 20 treatment preferably under pressure, with strong heat induration treatment, preferably after removal of the formed piece from the forming instrumentality.

During such heat induration treatment 25 the sulphur or other solidifying agent appears to act upon or with reference to certain of the other constituents of the material, particularly the solidifiable oil or the like, whereby the material of the piece is 30 transformed into a hard and durable condition, exhibiting superior strength with resistivity toward the action of chemical agents and solvents.

As typical of certain preferred methods of 35 producing the herein contemplated products, the following steps may be employed. Approximately 40 parts of stearine pitch and approximately 60 parts of asphalt are heated together to a temperature of approximately 500 degrees F. with stirring to effect 40 an intimate mixture of said ingredients. The mixture is thereafter cooled to approximately 475 degrees F., whereupon substantially 10 parts of castor oil is added and 45 the mixture again stirred. Thereafter the mixture is permitted further to cool to approximately 200 degrees F. and thereafter approximately 25 parts of benzol is added and the mixture again thoroughly stirred.

50 For production of a molding compound, approximately 286 parts of the aforescribed material, taken as a binder is thoroughly mixed and incorporated with approximately 1100 parts of a suitable filler such as asbestos, 66 parts of sulphur and 55 22 parts of iron oxide being added. Such mixing and incorporation of the foregoing ingredients may be facilitated by further additions of benzol up to or even somewhat 60 in excess of 100 parts. The mixture may be then disintegrated, screened and subjected to other desired known treatment preparatory to molding. Also it is preferable 65 that an appreciable interval of time, as for example twelve hours intervene be-

tween compounding of the molding material and actual pressing thereof. The material may be pressed in cool or cold dies under conditions similar to those ordinarily imposed in treatment of analogous molding 70 mixes. Following molding the material is subjected to strong heat treatment which may cover a period of hours up to or even beyond 24 hours at temperatures which are preferably elevated gradually from approximately 200 degrees F. to a final temperature 75 of about 500 degrees F.

Pieces produced in the manner aforescribed are characterized by very superior strength and resistance to impact. Also it 80 has been found that such pieces undergo in general lesser and more uniform degrees of shrinkage during cure than do pieces formed of materials prepared in the ordinary ways, whereas the pressing qualities of 85 the material are found to be superior.

While the aforementioned proportions of the various ingredients, particularly the stearine pitch and asphalt, have been found to be desirable and advantageous, it is nevertheless to be understood that such proportions may vary rather widely, whereas, for certain special purposes radically different proportions may be found desirable. Further in special cases it has been found possible and also desirable to reduce the quantity of the asphalt practically or even actually to the point of elimination thereof, whereas for other purposes it has also been found desirable similarly to decrease the 100 stearine pitch content.

Thus a compound may be produced by mixing together, at approximately 475° F., 800 parts of asphalt and approximately 82 parts of castor oil, the mixture being permitted to cool to about 200° F., and about 320 parts of benzol being thereafter added with stirring.

Approximately 286 parts of the last described compound, taken as a binder, together with 1100 parts of asbestos or other suitable filler, 66 parts of sulphur, 22 parts of iron oxide and either with or without further additions of benzol up to or even somewhat beyond 100 parts may be subjected to form giving treatment as aforescribed with strong heat induration treatment, preferably after removal of the 110 formed piece from the die or mold.

Also in each of the foregoing examples the 120 proportion of the solidifiable oil or the like may be varied between relatively wide limits.

Thus an advantageous compound characterized by high plasticity, superior molding 125 properties and relatively low and uniform shrinkage during induration may be produced by treating, in the manner described in the first of the foregoing examples, approximately 50 parts each of stearine pitch 130

and asphalt, together with approximately 20 parts of castor oil and a suitable quantity of benzol or the like and having incorporated substantially the proportions of filler material and sulphur mentioned in the previous examples.

Such compound is well adapted to form giving treatment and strong heat induration.

10 It is of course to be understood that the proportions of the various ingredients stated in each of the foregoing examples are capable of considerable variation to adapt the product to special conditions and uses.

15 It is also to be understood that the terms "stearine pitch", "asphalt" and others employed herein are intended to designate the substances obtainable commercially.

What I claim as new and desire to secure 20 by Letters Patent is:—

1. Composition material adapted to the plastic art, comprising, approximately, 40 parts of stearine pitch, 60 parts of asphalt, 10 parts of castor oil and 25 parts of benzol, 25 said material being capable of treatment under influence of heat without involving precipitation of a deleterious quantity of free carbon.

2. A hard and substantially infusible and 30 insoluble substance which is the heat induration residuum of material comprising a binder formed of approximately 40 parts of stearine pitch, 60 parts of asphalt, 10 parts of castor oil and 25 to 100 parts of benzol, 35 286 parts of said binder being mixed with about 1100 parts of asbestos, 66 parts of sulphur, and 22 parts of iron oxide, said binder being capable of treatment under influence of heat without involving precipitation of a deleterious quantity of free carbon.

40 3. The process of producing composition material adapted to the plastic art, which comprises melting and mixing together about

40 parts of stearine pitch and 60 parts of asphalt, cooling the mixture and adding thereto a solidifiable oil, further cooling the mixture and adding thereto a volatile solvent, said mixture being capable of such treatment without involving precipitation 45 of a deleterious quantity of free carbon, incorporating with the mixture an inert filler material, and incorporating an agent adapted under influence of heat to promote induration of the product. 50

4. The process of producing composition material adapted to the plastic art which comprises melting and mixing together about 40 parts of stearine pitch and 60 parts of asphalt, cooling the mixture and adding 60 thereto 10 parts of a solidifiable oil, further cooling the mixture and adding thereto at least 25 parts of a volatile solvent, said mixture being capable of such treatment without involving precipitation of a deleterious 65 quantity of free carbon, incorporating with about 286 parts of the mixture about 1100 parts of an inert filler material, and incorporating about 66 parts of an agent adapted under influence of heat to promote induration 70 of the product.

5. The process which comprises mixing together under conditions of temperature control about 40 parts of stearine pitch, 60 parts of asphalt, and 10 parts of a solidifiable oil, said mixture being capable of such treatment without involving precipitation of a deleterious quantity of free carbon, incorporating with about 286 parts of the mixture about 1100 parts of a relatively inert 75 filler, introducing about 66 parts of sulphur and at least 25 parts of a volatile solvent, subjecting the product to a cold molding operation, and indurating the formed articles by strong heat treatment. 80

In witness whereof, I have hereunto subscribed my name.

CLETUS F. CHOSA.